

# UNITED STATES PATENT OFFICE.

ISADOR LADOFF, OF WILKINSBURG, PENNSYLVANIA, ASSIGNOR OF THIRTY ONE-HUNDREDTHS TO WALTER D. EDMONDS, OF BOONVILLE, NEW YORK.

## METHOD OF MAKING ALLOYS.

1,221,874.

Specification of Letters Patent. Patented Apr. 10, 1917.

No Drawing.

Application filed February 25, 1916. Serial No. 80,393.

*To all whom it may concern:*

Be it known that I, ISADOR LADOFF, a citizen of the United States, residing at Wilkinsburg, in the county of Allegheny and State of Pennsylvania, have invented certain new and useful Improvements in Methods of Making Alloys, of which the following is a specification.

My present invention relates particularly to the making of such alloys as that for example known as "high speed steel," which depend for their utility and perfection upon alloy incorporation with a ferro metal of as definite respective quantities and proportions as possible of a plurality of certain rarer, harder, and more difficultly workable metals, these being, in this instance, tungsten, chromium and vanadium, the which respectively contribute to impart to the so called steel final product well known desired characteristics and behaviors, such as superior hardness, tensile strength, resistance, etc., and the objects of my invention comprise provision of procedures whereby a suitable alloy of such rarer metals, and, by aid thereof such final products can be produced with greater economy, certainty, and by less highly skilled labor than formerly.

I believe that hitherto in the manufacture of high speed steel for example, it has been the invariable practice to add to the predominant molten ferro metal bath separately, the preliminarily separately produced binary alloys of ferro metal, iron for example, and respectively tungsten, chromium, vanadium in, as nearly as could be thus produced and ascertained, the desired proportions. This procedure has not only involved three separate preliminary operations for production of the three separate alloys thus employed, but also difficulty in uniformly producing successive batches of each of said alloys in desired identity of composition, and consequent difficulty in sufficiently accurately calculating and weighing the respective quantities of each of said alloys to be separately added to the bath of ferro metal under treatment. Moreover, the degree and amount of heat required for proper melting or dissolution of these separately produced binary ferro alloys of these rarer, more refractory metals have proved undesirably expensive, and the relatively long time required, and relatively

extensive surfaces of said separately added alloys exposed during the relatively long time required to so melt them, has undesirably exposed said rarer metals to oxidation, etc., and undesirably promoted segregation of resulting compounds and gases in the charge and final product. 60

My present invention is based upon my discovery that the aforesaid, and other difficulties and imperfections of previous practice can be greatly ameliorated, or for the most part entirely overcome, by the preliminary production of a single alloy of ferro metal with all of the said rarer and more refractory metals to be added to the ferro bath in order to produce the desired final product. 65

Thus, in the manufacture of high speed steel, I preliminarily produce a quaternary alloy of iron with tungsten, chromium and vanadium, each of the three last mentioned metals being in the respective interrelated proportions and total quantity required for the particular operation and final product in view, and this quaternary alloy of which 75 the said rarer metals in their aggregate should preferably constitute not less than at least fifty per cent. I then add, to the ferro bath to be treated, in quantity calculated to impart to the latter sufficient of said 80 rarer metals, in required respective proportions. 85

I have further discovered that, for the purpose of adding it to a bath of ferro metal in the manufacture of high speed tool 90 steels, the aforesaid preliminary, quaternary, alloy of ferro metal with tungsten, chromium, and vanadium is more effective, more economically made, and with greater 95 certainty as to proportions, and with more effective and superior results by such direct reduction methods at temperatures lower than those of fusion of the respective metals, as are disclosed, or claimed, in Letters Patent No. 1,040,699, and No. 1,042,694, granted 100 to me respectively on the 8th day of October, 1912 on the 29th day of October, 1912, and in my pending application for patent Serial Number 55,418, filed October 12, 1915.

Such metals may be summarized as consisting essentially of commingling the oxids of the respective metals and in presence of a carbonaceous agent reducing them at temperatures lower than those of fusion of the 105 said metals. 110

By my said methods of producing my preliminary quaternary alloy, I have much better control, quantitatively as well as qualitatively, of all the constituents of the alloy, and produce it with less temperature cost, and with less risk of segregation at any stage of the entire process.

My said preliminary produced ferro alloy containing the said three other metals, in required proportions, I incorporate in required quantity into the usual crucible-contained, molten, ferro bath under treatment, and containing the usual more or less pure iron, carbon, manganese, etc. After maintaining the usually required temperatures sufficiently long, and high, to insure melting of the thus added alloy and its dissolution in the bath, the resulting melt is teamed, cast, or otherwise treated as usual to produce the desired final product.

By my present invention above described, I attain, among other things, the following advantages, viz: dispensing with all but one operation in production of ferro alloy with the said rarer metals; also economy in heat required, I having also discovered that it requires less expenditure of energy to produce my one multiplex ferro alloy with the said three more refractory metals than to produce a binary alloy of one only of such metals with a ferro; also avoidance of oxidation, and of formation of segregation-inducing deleterious compounds or gases in the bath treated, and in the final product, due to my single quaternary alloy melting or dissolving more rapidly and at lower tem-

peratures than any binary alloy such as formerly employed; and particularly also to the fact that the surface presented to oxidation by my multiplex alloy in comparison to its weight and volume, is, other things being equal, less than those of an equivalent number and quantity of binary alloys.

What I claim as new and desire to secure by Letters Patent is the following, viz:

1. The method of making high speed tool steel which comprises preliminary producing at a single heat, a quaternary alloy of a ferro metal with tungsten, chromium and vanadium, and of which alloy the said tungsten, chromium and vanadium constitute, in their aggregate, not less than fifty per cent., and thereafter melting the said alloy in a bath of ferro metal not comprised in said alloy.

2. The method of making high speed steel which comprises commingling with a ferro-metal or its oxid oxides of tungsten, chromium, and vanadium, reducing said oxides to metallic state at temperatures below that of the melting points of their respective metals, and thereafter melting the resulting alloy in a bath of molten ferro-metal.

3. An alloy comprising a ferro-metal, tungsten, chromium and vanadium, and of which its aggregate of tungsten, chromium and vanadium constitutes over fifty per cent.

ISADOR LADOFF.

Witnesses:

A. M. Coos,  
JAS. E. SWISSELM.